

May 12, 1936.

M. FRÄNKEL

2,040,650

ORE SMELTING AND REDUCTION PROCESS

Original Filed Oct. 14, 1931



INVENTOR

MATHIAS FRÄNKEL

BY

Watson, Bristol, Johnson & Leavittworth

ATTORNEYS

## UNITED STATES PATENT OFFICE

2,040,650

## ORE SMELTING AND REDUCTION PROCESS

Mathias Fränkl, Augsburg, Germany, assignor to  
American Oxythermic Corporation, New York,  
N. Y., a corporation of Delaware

Original application October 14, 1931, Serial No.  
568,710. Divided and this application July 19,  
1935, Serial No. 32,354. In Germany February  
4, 1931

2 Claims. (Cl. 75—92)

The invention relates to a smelting process for the treatment of ores, metals and minerals, as well as to the reduction of ores and to the preparation of compounds of metallic elements. It particularly relates to a process for the manufacture of carbides, and includes correlated improvements and discoveries whereby and where-with such process may be enhanced.

An object of the invention is to provide a process for smelting and preparation of compounds of metallic elements wherein the normal gas flow is supplemented or intensified by an augmented gas circulation.

A further object of the invention is to provide a process in which the yield is increased through augmented gas circulation and combustion of carbon with highly concentrated oxygen.

A still further object of the invention is to provide a process in which the gas flow is increased by a regenerative cyclic process without a lessening of the quantity of useful heat in the region requiring high temperature.

Other objects of the invention will in part be obvious and will in part appear hereinafter.

The invention accordingly comprises the several steps and the relation of one or more of such steps with respect to each of the others thereof, which will be exemplified in the process herein-after disclosed, and the scope of the invention will be indicated in the claims.

For a fuller understanding of the nature and objects of the invention reference should be had to the following detailed description taken in connection with the accompanying drawing, in which there is depicted an apparatus suitable for the production of compounds of metallic elements, as carbides and ferro-alloys, as ferro-silicon, in which the operation is effected wholly within the regenerators.

The practice of the invention, accordingly, involves first establishing the conditions for carrying out the smelting operation, and more particularly by smelting the charge of material with utilization of solid fuel containing regenerators. The material is charged directly into the regenerators along with the solid fuel content whereby use of a separate furnace charged with material is obviated and the charge then smelted by means of heat generated by combustion of the contained fuel in one regenerator, the gas so produced being then conducted through a second regenerator in which charged material is smelted and contained fuel preheated, and alternately and periodically reversing the flow of gases through the regenerators. More especially the process may

be carried out by finely sub-dividing the material to be treated, and introducing such material into the high temperature zone of one of the regenerators by blowing. The smelting is thereby effected by heat generated as above described.

In the production of ferro-silicon, for instance, the whole operation is effected within the regenerators A' and A'', as shown in the drawing. In this case an amount of ore or scrap iron which, compared with the amount of fuel is in every case very small, together with the appropriate quantity of silicic acid in the shape of sand or gravel, may be charged through the regenerators or blown in in a crushed state through the nozzles d, together with oxygen. Crushed or ground turnings or drillings are most suitable for this purpose.

If in place of ore or iron, limestone or burnt lime is charged into the regenerators from the top or blown in in powder form at the bottom, then at the high temperature prevailing carbon and lime will combine to form carbide of calcium.

If neither iron nor lime is supplied, but silicic acid in the shape of sand, then carbide of silicon is produced (grinding material).

In the same manner charged alumina may be reduced to aluminum carbide.

Oxygen, together with crushed coal and crushed lime, or sand or crushed iron scrap is blown in through the nozzles d if such material is not charged into the regenerators from the top.

The second phase of the invention supplements the previously described process by a regenerative cyclic process for increasing gas flow in the smelting space, without lessening the quantity of useful heat in the region of high temperature.

Through the nozzles d oxygen containing less nitrogen than the air is introduced. A blower e serves to cause gas to circulate from one regenerator to the other and across the smelting space in such manner that alternately gas is withdrawn from one regenerator and blown through the other into the smelting and reducing zone and at the same time removed therefrom by the first regenerator. After a few minutes' blowing time the direction of the gas stream is reversed by means of the hinged valves k' and k'' and the gas withdrawn from the regenerator which previously functioned to heat the gas being introduced into the smelting space.

While streaming from the bottom to the top, the gas gives up its heat to the fuel content of the one regenerator; on the way down it takes it up again. The blower e thus withdraws only cooled gas, as the temperature of the coal con-

tent of the regenerators drops from bottom to top and remains at the top end at about 20 to 30° C., while at the bottom end it may be as high as the required smelting temperature, that is, from 5 1300 to 2500° C. Before entering the circulation blower the cycling gas may be cooled, e. g., to the temperature of cooling water, and when this is done the temperature of the regenerators at the top end may be correspondingly raised. This 10 cooling may be effected by conducting gas through a water cooler X, prior to its passage to the blower e.

Coke is a suitable fuel for filling the regenerators. However, since coke as a fuel is more expensive than coal, the needed heat is advantageously procured by using mainly burning-dust or fine coal, which is blown in through double nozzles, together with oxygen, or separately. 15 A small portion, about 10%, of the coke filling of the regenerators must, however, always be burned also, because otherwise the nozzles would soon be clogged by the dust contained in the cycling gas. The burned portion of the coke filling must then be replaced by putting in a corresponding 20 amount at the top.

In a large number of metallurgical processes of the high temperature class, however (ore smelting) and also in the production of compounds of metallic elements (carbides), or of 25 ferro-alloys (ferro-silicon) only a small part of the total amount of heat required is utilized for preheating the charge to reducing temperature, a much larger part is used to attain a temperature which lies above the smelting point of raw 30 iron and slag; that is, above 1300° C. In the production of carbides and ferro-silicon, the limit lies higher still, that is, at 1600 to 2000° C.

If this heat is to be produced by combustion (instead of electro heat), then only that part 40 is utilizable for this purpose which is generated above that temperature, because the heat contained in the flue gas and which is below the reducing and smelting temperature, is lost for the reducing and smelting process.

45 By burning one kg. carbon to CO only 2430 cal. of heat are liberated. The combustion with air, theoretically, gives a temperature of 1650° C., which is raised to about 2450° C. if the air supplied is heated to 800° C. Hence the utilizable 50 quantity of heat in the smelting zone of the furnace is 1650—1300=350:1650, or 2450—1300=1150:2450, that is, about one fifth to one half of the heating value of the carbon. To gain more 55 than one fifth the quantity of utilizable heat, the excess above one fifth must be supplied at the cost of air heating.

If, in comparison, nitrogen-free oxygen is used for the combustion, a theoretical combustion temperature is generated of about 8000° C., and the 60 relation of useful heat to waste heat will be 8000—1300=6700:8000, that is, about four fifths.

The advantageous features of the invention may be thus summarized:

1. The operation of a smelting furnace as hereinbefore described is supplemented by a regenerative cyclic process;

2. A quantity of gas is blown across alternately from left to right and in the reverse direction, through two regenerators which are filled with a 70 fuel used as a heat storing material, whereby the sensible heat of these gases is alternately taken up by the fuel filling of one of the two regenerators and, at the same time, given up by the other to the circulating gas, so that the blower may be

operated within the limits of admissible temperature, and in order to increase gas flow in the smelting space;

3. The high combustion temperature obtained when operating with highly concentrated oxygen 5 is lowered by a circulating gas to an admissible degree, without lowering the total heat in the high temperature zone below that of operation at maximum temperature;

4. That by burning the fuel content of the 10 heat storing regenerator in the high temperature zone and renewing the fuel filling at the upper and colder end of the regenerator, the requisite continuous renewal of the heat storing material (regenerator contents) is effected while 15 avoiding clogging by the dust contained in the circulating gas or by slagging;

5. Only a small amount of the expensive fuel used as filling material for the regenerators need be burned to prevent clogging, and the requisite 20 heat, in the main is generated by blowing coal dust or small coal into the zone of combustion; and

6. That either the regenerators are charged with the material to be smelted or such material 25 is crushed and blown directly into the smelting zone, either through the oxygen nozzles or through special nozzles.

This application is a division of my copending application Serial No. 568,710, filed October 14, 30 1931.

Since certain changes may be made in carrying out the above process without departing from the scope of the invention, it is intended that all matter contained in the above description shall 35 be interpreted as illustrative and not in a limiting sense.

It is also to be understood that the following claims are intended to cover all of the generic and specific features of the invention herein described, and all statements of the scope of the invention which, as a matter of language, might be said to fall therebetween.

Having described my invention, what I claim as new and desire to secure by Letters Patent is:

1. In a process for smelting a charge of material utilizing solid fuel containing regenerators, the improvement which consists in charging the materials to be treated directly into the regenerators whereby the use of a separate furnace charged with material is obviated, and smelting by means of heat generated by combustion of contained fuel in one regenerator, the gas so produced being then conducted through a second regenerator in which charged material is smelted and contained fuel preheated, and alternately and periodically reversing the flow of gases through the regenerators.

2. In a process for smelting a charge of material utilizing solid fuel containing regenerators, the improvement which consists in finely subdividing the material to be treated, introducing said material into the high temperature zone of one of said regenerators by blowing, smelting by means of heat generated by combustion of contained fuel in said regenerator, the gas so produced being then conducted through a second regenerator in which contained fuel is preheated and alternately and periodically reversing the flow of gases through the regenerators, and correspondingly introducing the material alternately into the regenerators.

MATHIAS FRÄNKEL.